

## UNITED STATES PATENT OFFICE.

ANDRÉ MOUILLEFARINE, OF PARIS, FRANCE.

## DIELECTRIC SUBSTANCE AND PROCESS FOR MANUFACTURING SAME.

No Drawing. Application filed February 18, 1927, Serial No. 169,420, and in France February 18, 1928.

This invention has for its object to provide a new product possessing dielectric properties equal to or higher than those of the best insulating substances as used in the industry particularly in appliances utilizing high frequency electric currents, said new product being obtained by a simple, expeditious and cheap process from suitably selected wood by treating the latter by means 5 of one or several solutions adapted to free same from the whole of its contents of non-insulating substances and by a physico-chemical transformation of its contexture to render the whole of its mass absolutely and in- 10 variably dielectric.

Numerous attempts have been made heretofore to manufacture particularly from wood, a material easy to obtain at low cost and in large quantities industrially, insu- 20 lating substances i. e. substances capable of withstanding without any substantial losses low or high tension electric currents or dielectric substances i. e. substances capable of similarly withstanding high frequency elec- 25 tric currents whereby such substances might be used to supersede the best solid dielectrics such as ebonite, vulcanite, bakelite, indiarubber, etc. Such attempts failed to give satisfactory results as the insulating substances 30 thus manufactured only had fairly bad dielectric properties which moreover dwindle down in the long run particularly when hy- grometric or other ambient conditions are unfavorable.

Moreover it is a fact that the most perfect dielectric at present known being simply atmospheric air, attempts have been made in the course of the aforesaid experiments to create and manufacture certain light insu- 40 lating agglomerates i. e. substances containing under a small weight a large number of pores that is to say of cells or small pock- 45 ets full of air, the conductivity of said agglomerates being in an inverse ratio to the number of these air cells since their multi- 50 plicity increases, as self-explanatory, the dielectric capacity of these agglomerates. However none of such attempts has so far led to the industrial solution of the problem.

Now the present invention relates to a new product utilizable instead of ebonite, vulcanite, bakelite, indiarubber or analogous materials, either as an insulation or as a dielectric substance, said product being ob- 55 tained directly from woods of suitably se-

lected species and qualities and adapted to be dyed dark brown or black so as to mistakenly acquire the appearance of ebonite. It also relates to a physico-chemical process—inseparable from the said new product—whereby this dielectric substance may be manufactured industrially from these woods, said process essentially consisting, firstly, to eliminate from the numerous vessels or cells of the vascular tissue of the 60 wood (either primary or secondary) all their moist materials or more generally all materials making up its ligneous structure and which to various extents are conductive so as to merely leave a fibrous and porous 70 carcass constituting by itself an insulating armature and, secondly, to fill up or stuff by capillarity the channels thus formed throughout the fibres of the said tissue by means of a filling mass composed of one or 75 more highly insulating substances such as certain substances obtained from bituminous shales whereby the former cells of the wood previously emptied out of their conductive materials become filled up to regulatable de- 80 grees of saturation with said extraneous insulating substance or substances and thus their dielectric function is, as it were, multiplied by the insulating and supporting 85 function of the said carcass or armature.

One feature of this process resides in the fact that the wood having been suitably selected and cut up is first optionally submitted (in case the dielectric substance must re- 90 semble ebonite) to a dyeing bath and left 95 therein until it has acquired right to the heart for instance the fine black colour of ebonite and is afterwards immersed into one or several other baths containing substances obtained from bituminous shales which si- 100 multaneously open out its vessels and cells and by completely eliminating therefrom the several conductive materials and fills them with an insulating mass which by capillarity or osmose percolates through the whole mass of the wood owing to its fibres being now open and distended and thus gives same the required dielectric qualities.

Other features of this process and the new dielectric substance obtained therefrom will 105 be apparent from the following description which relates, by way of example, to an in- 110 dustrial method of carrying it out.

According to this method and assuming that the dielectric substance to be obtained 115

should simulate ebonite, cut up pieces of a suitably selected wood having fine pores such as chestnut or witch wood (the category of wood: primary wood, secondary wood, heart, sap wood, etc., having no bearing provided its pores are sufficiently small) are first submitted to a black dyeing bath composed for example of the admixture of the following materials:

|                    | Grams. |
|--------------------|--------|
| Basic black        | 10     |
| Acetic acid        | 10     |
| Chloride of sodium | 5      |
| Water              | 975    |

whilst effecting this dyeing operation in the usual dyeing conditions during about 24 hours, the temperature being maintained at about 100° C. during the first 4 hours where-  
 20 after the bath is allowed to freely cool whilst the wood soaks therein during the remaining 20 hours. Then, after having caused the wood dyed in the aforesaid way to drip out by exposing same to the open air during  
 25 about an hour or, if it is desired to hasten its drying, by exposing same to one or several hot draughts (for example in a dry kiln) the pieces or logs of wood are im-  
 30 mersed in a liquid mass composed of one or several insulating substances obtained from bituminous shales such as ozokerite, naph-  
 tadi, hatchettin or mineral tallow previously molten by first heating the same rapidly to 150° C. which temperature corresponds to  
 35 the immersion of the wood therein, then pro-  
 gressively up to 300-350° C. The wood is left in this hot liquid mass for approxi-  
 mately 3 to 4 hours so that it becomes sat-  
 40 urated with the said insulating substances to the approximate extent of 80 to 90% whilst maintaining said mass at the aforesaid tem-  
 perature of 300-350° C. and afterwards withdrawn and allowed to dry naturally in cold air. It is then only sufficient after  
 45 having wrought it to the desired shape. (by sawing, turning or otherwise) to varnish it to give it its final finish and polished state, for instance by making use of a varnish composed of:

50 Shellac-----35 kgs. (about 77 lbs.)  
 Spirit (80 to 90°)-----100 kgs. (about 220 lbs.)

After being thus varnished by the usual methods and at a temperature of about 14° to 16° C., the pieces of wood either wrought or non-wrought and entirely unrecognizable and having the true appearance of ebonite have a dielectric power which is at least equal to that of the latter substance and are

thus readily utilizable for several electrical 60 applications involving the use of ebonite.

By the operative method that has just been described it is possible to obtain a high grade dielectric substance having the above- 65 cited properties. Said method has however only been given as an example of the way the invention can be carried out as it is self- explanatory that the application of its principles will necessarily vary according to the working conditions and particularly to 70 the species and quality of the wood treated, said principles involving in all cases a physico-chemical treatment consisting, after optionally dyeing the wood to the heart (ex- 75clusively for giving the wood for instance 75 the black colour that will make same ebonite- like, it being naturally possible to do away with such dyeing step for example in cases where the dielectric substance should keep the natural tint of the wood), to eliminate 80 from its fibres all conductive materials contained therein whilst opening them out for enabling them to be thoroughly penetrated in the same operation by fluid insulating sub- 85 stances in such proportions as will stuff or cram all empty cells of the opened out or porous structure or carcass thus obtained. Within the scope of such directive principles and in as far as the essentiality of the above- 90 cited operative conditions is not modified, the selection of materials, the duration, the temperature or the other operative factors may be varied without departing from the domain of the invention.

What I claim is:

The herein described process of rendering wood dielectric, which consists first in dyeing the wood to resemble ebonite, comprising the step of immersing the wood in a liquid mass composed of basic black, acetic acid and sodium chloride for substantially twenty-four hours, the first four hours of which the mass is heated to 100° C. and for the remaining time the mass is permitted to cool, thereafter submitting the wood to a heat treatment, 105 then to the action of an insulating mass consisting of bituminous shales which first opens up the pores of the wood by removing all conductive substances therefrom and then replaces the discharged conductive substances, the action taking place during a change in temperature of the mass from 150° C. to 300° C. or more, thereafter drying the 110 impregnated wood and finally finishing its surface with shellac bearing varnish. 115

In testimony whereof I affix my signature.

ANDRÉ MOUILLEFARINE.